

## UNITED STATES PATENT OFFICE

LESTER KIRSCHBRAUN, OF LEONIA, NEW JERSEY

## AQUEOUS DISPERSIONS AND PROCESS OF MAKING SAME

No Drawing.

Application filed December 15, 1927. Serial No. 240,337.

This invention pertains to aqueous dispersions of substances normally immiscible with water and to methods of producing the same. More particularly the invention relates to 5 dispersions in which the said substances comprise the internal phase, the water being in the external or continuous phase.

The invention is more particularly concerned with aqueous dispersions of such substances as are made by effecting the dispersing action with the aid of organic colloidal materials such as gelatine, tapioca flour, wheat flour, dextrine, starch, starch-containing substances and the like.

15 It has been found, for example, that certain colloids of this type may be satisfactory for use as dispersing agents in the production of bitumen-pitch type dispersions, providing the dispersing operation is carried on in such 20 manner that the dispersed particles are maintained as the dispersed phase throughout the dispersing action.

Dispersions as thus produced are highly 25 stable in the presence of acids, alkalis, powdered pigments, hydraulic cement, and the like, and such dispersions are also suspensible over long periods of time and possess other desirable properties.

One of the objects of the present invention 30 is to provide a method in which the dispersing action with the aforesaid materials may be facilitated, and the resultant product improved as to fineness of particle size, "body", and use of minimum quantities of dispersion means.

While the size of the dispersed particles resulting from the dispersion of bitumen-pitch 40 type materials with dispersing agents of the type indicated, is sufficiently fine for most purposes, nevertheless, in some instances, a much finer degree of subdivision is desired, and it is accordingly another object of the present invention to provide methods where- 45 by the above named colloids may be employed for producing dispersions in which the particles dispersed are of an exceedingly fine order of subdivision, as a result of which the finished product possesses a much finer 50 and longer body than is obtainable with such

dispersing agent when used without the improved treatment presently to be described.

One of the characteristics of dispersions made with certain of the above named colloids is that when such dispersions are employed as coatings and applied in the form of films, the removal of the water and the consequent coalescence of the dispersed particles results in a film which is characterized by a certain degree of tackiness. This tackiness is in certain instances desirable as providing adhesive qualities which adapt the film for use as a bonding coat. Under other conditions of use, however, it is desirable that the dried water-free film of the dispersion be free of tackiness and hence another object of the present invention is to produce dispersions of this type in which the dispersed particles are much finer than are ordinarily attainable and which are capable of drying to a continuous non-tacky and substantially impermeable film.

The foregoing objects are achieved by treating the colloid used as the dispersing agent in the manner to be hereinafter described in more detail.

In carrying out the invention tapioca flour or any of the common forms of starch, as for example, corn starch, potato starch, or the like, may be employed as the dispersing agent. The substance to be dispersed may comprise any solid or semi-solid bitumen such as asphalt, either of the native or artificially prepared variety, resins, pitches, rubber, or the like, all embraced in the term "bitumen-pitch type". Where the material to be dispersed is a solid or semi-solid bitumen it may be preferably heated so as to be brought to a fluid condition. The temperature at which the bitumen may be maintained during the process of dispersion may vary over a considerable range, depending upon the character of the bitumen. Where starch is selected as the dispersing agent, the same may be preferably conditioned by forming a swollen paste thereof in water.

In one mode of carrying out the invention, for example, tapioca flour may be cooked into a paste with about three (3) times its weight of hot water. The concentration of 100

the flour may vary, however, over a considerable range depending upon the thickness desired in the pasty mass. The swollen paste as thus produced may then be employed as the dispersing media for assisting in the dispersion of the bitumen. The dispersing action may be carried out in any suitable form of agitating mechanism adapted to cause rapid agitation of the mass contained there, in so as to effect the necessary subdivision of the bituminous material, the particles being thereby dispersed and maintained in suspension in the aqueous phase. The dispersing apparatus may be of a type provided with agitating propellers, or it may be of any other suitable type. The dispersing apparatus may be preferably provided with any suitable means, such as water jackets or the like for regulating the temperature of the mass being treated therein.

It is preferable in conducting the process as a batch operation, to add the heat-liquefied bitumen to the flour paste and to continue the addition of bitumen during the agitation of the mass until the desired amount of bitumen has been dispersed in the form of finely divided particles.

I have found in accordance with one phase of the present invention, that if the paste of the organic colloidal material is treated with an acid or acidic salt, that the dispersing action is thereby facilitated so that the desired end product may be more readily produced. For this purpose I may add to a starch paste, for example, acids such as hydrochloric, acetic or sulfuric, or such acidic salt as potassium dichromate, aluminum sulfate, or the like. The amount of acidic substance added should generally be sufficient to bring the hydrogen ion concentration of the starchy paste to a value of, say 4.0 to 5.0. At this range the dispersion of the base is more readily accomplished than when using a paste made with untreated starch.

When producing dispersions of this type with pastes made, for example, with carbohydric colloids, such as starch or starch-containing materials in their untreated state, the mass being subjected to the agitating or dispersing action is preferably maintained in a pasty condition, but the mass should not be permitted to become so thick as to cause the formation of coarse grainy particles or the coalescence of the dispersed particles.

I have found, however, in accordance with another feature of the present invention, that if relatively small quantities of a tannin-containing material or material functioning as does tannic acid in this respect is present, a very superior type of dispersion may be produced by virtue of the fact that the presence of said material permits the process to be carried on under such conditions that the mass undergoing dispersion is maintained in

a relatively thick pasty condition. Under such conditions of operation the high internal viscosity of the thick mass assists the dispersing action materially so that the particles are dispersed in an exceedingly fine state of subdivision such as is not attainable where the operation is carried on while the viscosity of the mass is maintained relatively thin. The dispersion as thus produced is not only finer as respects the size of the dispersed articles, but in most cases it is also more smoothly and heavily bodied than the dispersion made with the untreated starch paste.

One type of material which I have found suitable for this purpose is tannic acid and tannin-containing substances such as tannic extracts, as for example, quebracho.

The tannin-containing or tannin-like material may, if desired, be incorporated during the dispersing action, but better results are had by mixing the tannic acid or tannin-containing substance with the said colloid and carrying on the dispersion with this mixture. In the latter case, the tannin-containing material may be preferably subjected, together with the dispersing agent, to the action of hot water, whereby to form thereof a thick viscous paste.

I have found that very small quantities of the tannin when mixed with starch are sufficient to accomplish the purpose of the present invention. The quantities of tannic acid may range from, say 1% by weight of the starch to 10%, more or less, by weight thereof. Larger quantities are to be avoided because of the resultant tendency to harmfully affect the dried film of the product. Where it is desirable to eliminate the tackiness which usually characterizes the dried film of dispersions made with carbohydric colloids, this may be accomplished with larger amounts of tannic acid within the range given above.

As a specific embodiment of this invention, a mixture may be made of 10 parts of corn starch with .2 parts of tannic acid, the mixture being then formed into a plastic mass by boiling in 30-40 parts, more or less, of water. This plastic mixture may then be employed in the dispersion of Mexican asphalt of, say 100 to 200° F. melting point or other similar bituminous material, the operation being carried on in such manner that the bitumen is at all times retained as the dispersed phase. In this way it is possible to disperse asphalt of the character indicated in quantities ranging from 30 to 40 times by weight of the amount of starch and tannic acid in the plastic mixture comprising the dispersive media, the aqueous content of the final product constituting about 85-90% more or less, thereof. The dispersion thus produced may, therefore, comprise, say 1.5 to 2.0% starch, .015% to .05% of tannic acid, is substantially perfectly suspensible and very stable in the presence of alkalis,

acid salts, powdered pigments, mineral aggregate and the like, none of the latter causing any perceptible amount of flocculation of the dispersed particles or producing any 5 other objectionable effects in the dispersion.

Substantially similar results may be attained by substituting quebracho for the tannic acid. This extract contains compounds of tannin in amounts equivalent to about 35% 10 of its weight of tannic acid, and hence where this material is available it may be used in substantially the manner above set forth, and in quantities such that the tannin content thereof approximates the quantities of tannic 15 acid above specified. The product made with this material is substantially similar in all respects to the dispersion made as above described with tannic acid.

A dispersing agent such as gelatin also 20 lends itself very well to the above treatment with tannins or tannic acid, in which case the gelatin becomes insolubilized so that it is irreversible in the final water-free film.

The product thus produced may be used 25 as a protective coating with or without pigments and fillers. It may be mixed with mineral aggregates and used as a road binder. Fibrous materials such as asbestos or vegetable fibres may be incorporated readily 30 with it to produce plastic fibrous compositions capable of use for roofing or as a base for mastic flooring mixtures.

Rust inhibitive agents, either soluble or insoluble in the aqueous phase may be readily 35 incorporated into this dispersion without the occurrence of flocculation whereby to produce a coating readily adapted for protection of iron and steel.

By the term "tannin-like substance" as used 40 in the claims I mean tannic acid, tannin extracts, and substances generally functioning in the same manner as do these substances when used with an emulsifying agent of the type referred to in the foregoing description.

45 I claim as my invention:

1. The herein described process of producing an aqueous bitumen-pitch type dispersion, which comprises making an aqueous paste of a carbohydric colloid, adjusting said 50 paste to a pH value of 4.0 to 5.0, by a tannin-like substance and dispersing a bitumen-pitch type base with said adjusted paste.

2. An aqueous bitumen-pitch type dispersion comprising by weight at least substantially 55 60% of bitumen-pitch type base, 1.5% to 2% of a paste-forming carbohydric substance, 0.015% to 0.2% of a tannin-like substance, and the balance water.

3. An aqueous bitumen-pitch type dispersion comprising by weight at least substantially 60% of bitumen-pitch type base, 1.5% to 2% starch, 0.015% to 0.2% of a tannin-like substance, and the balance water.

In testimony whereof I affix my signature.